

# UNITED STATES PATENT OFFICE.

FREDERICK WILLIAM DOBSON, OF TAMWORTH, ENGLAND.

## METHOD OF BLEACHING CELLULOSE WOOD-PULP.

1,104,109.

Specification of Letters Patent.

Patented July 21, 1914.

No Drawing.

Application filed January 26, 1912. Serial No. 678,656.

*To all whom it may concern:*

Be it known that I, FREDERICK WILLIAM DOBSON, a subject of the King of Great Britain and Ireland, and resident of Tamworth, Staffordshire, England, have invented a certain Improved Method of Bleaching Cellulose Wood-Pulp, of which the following is a specification.

This invention refers to the bleaching of wood pulp fiber as used in paper making and commercially known as chemical wood cellulose, which is wood treated by chemical reducing agents. Usually chemical wood cellulose is bleached in large open trough-like vessels, the cellulose, which is in sheet form, being first broken up and then placed, along with a supply of water to soften it, into the bleaching vessels. To the cellulose is added the bleaching liquor which is in a dilute form, there being a large excess of water. The cellulose and bleaching liquor are then circulated around and around the vessels until the cellulose is fully bleached. The drawbacks to this method of bleaching are that the time taken for bleaching is usually very considerable; that owing to the vessels being open the pulp is liable to get contaminated with dirt, etc.; that the fumes from the bleaching materials, which are injurious to health, are free to escape into the atmosphere; that the bleaching materials cannot be regulated to any degree of nicety for a given bleach and that the cellulose, after bleaching, requires to be passed through drainers to drain off the surplus liquor before it can pass to the beaters, this latter being a serious drawback when rapidity of output is of first importance.

This invention has for its object a method of bleaching chemical wood cellulose whereby the aforesaid drawbacks are overcome, and especially in respect to the bleaching of the same quantity of pulp in less time than heretofore and also in respect to dispensing with the need to drain the cellulose after being bleached and before passing to the beaters.

According to the invention, the improved bleaching operation is carried out in a closed vessel, preferably of drum formation, and capable of being rotated. Usually an iron or steel vessel similar to a horizontal keir will be used, the vessel being supported horizontally by trunnions rotating in fixed bearings. Upon its interior the vessel may

be faced or lined with cement, tiles or other facing or lining capable of protecting the vessel from the action of the bleaching liquor. This lining is not strictly necessary and may be omitted. Into such vessel, 60 which is provided with suitable manholes, is placed the cellulose and bleaching solution. In practice it is found best to first run the supply of bleach liquor which is in a concentrated form, into the vessel, and then the 65 water necessary for producing the desired bleaching solution. To this solution is then added the cellulose which is, preferably, in dry sheet form. That is to say, the cellulose is not previously broken up and is quite 70 dry when introduced into the vessel, no moisture of any kind having been applied to it. The bleaching material will be chlorid of lime. When charged with the proper 75 quantities of cellulose and bleaching solution, the vessel is slowly and continuously rotated, thereby causing the cellulose and bleaching liquor to become thoroughly intermixed and the desired bleaching operation to be effected in a comparatively short time. 80 The rapid bleaching operation is largely due to the cellulose being in a dry form on the bleaching liquor coming in contact with it, which enables the bleaching material to rapidly penetrate the cellulose. In other 85 words, the cellulose in a dry state rapidly absorbs moisture and by this invention advantage is taken of such fact to bring about the rapid bleaching operation.

A vessel suitable for the purpose of the 90 invention may be 24 feet long by 7 feet diameter, suitable pulleys or gearing being provided for transmitting rotary motion to the vessel.

There are different kinds of chemical 95 wood cellulose but this invention is concerned chiefly with sulfite cellulose and soda cellulose sold unbleached for bleaching.

The following examples of the proportions of concentrated bleaching liquor, 100 water and cellulose for a complete bleach have been found to give the most satisfactory results, viz:

(a) 2 tons of sulfite cellulose, 435 gallons of bleaching liquor ( $5\frac{1}{2}^{\circ}$  to  $6^{\circ}$  Twaddell), 105 1000 gallons of water. This represents 4.8 lbs. bleaching powder to 100 lbs. of dry cellulose.

(b) 30 cwt. of soda cellulose, 690 gallons of bleaching liquor ( $5\frac{1}{2}^{\circ}$  to  $6^{\circ}$  Twaddell), 110

630 gallons of water. This represents 10.2 lbs. bleaching powder to 100 lbs. of dry cellulose.

It is to be noted that soda cellulose expands on absorption with water more than sulfite cellulose and consequently reduces the holding capacity of the vessel, it also requires more bleaching solution to give the same degree of whiteness as sulfite cellulose.

10 The above examples of proportions are subject to variation according to temperature. For example, slightly less bleaching liquor is required in the winter, than in the summer. The above examples are for summer working. As aforesaid, the cellulose, should be introduced dry into the bleaching vessel. This is important as it enables the bleaching liquor to more readily penetrate the cellulose, the presence of any water previously added to the cellulose being detrimental to the rapid action of the bleaching liquor. For the quantities before named and the size of vessel indicated the bleaching of the cellulose is completed in about 3 20 hours, the vessel being rotated about 2 to 4 revolutions per minute.

After being bleached the cellulose is removed from the vessel through a manhole or manholes direct into tubs or other receptacles by which it may be conveyed to the beaters. That is to say, owing to a concentrated bleaching liquor being used and also owing to only so much bleaching liquor being used as is necessary, there is no need 30 for the bleached cellulose to be submitted to a draining operation, the bleached cellulose being in a condition suitable for direct transference to the beaters. It should now be seen that by reason of the rapidity and exactitude with which the bleaching operation can be performed and further by reason of the entire absence of the need for 35 drainers considerable advantages are obtained over and above the ordinary method 40 of treatment. Moreover, the plant and

power required for bleaching a given quantity of pulp in a given time are much less than formerly, thereby economizing floor space (which is often a great desideratum) and reducing the cost of bleaching. Further, the pulp bleached as aforesaid is cleaner and in a more satisfactory state than when bleached in open vessels. Another advantage is that as the bleaching liquor can be regulated in amount to the exact requirements, the bleaching material when removed from the vessel is practically free from smell. Further by treating the cellulose in sheet form the labor of breaking it up as heretofore necessary is avoided, and much 50 time thus saved. It will be understood that the amount of bleaching material used will depend on the degree of whiteness required.

The bleaching vessel will be driven by any suitable form of motor and the direction of its rotation may, by suitable reversing gear, be periodically reversed to insure of the most effective action of the bleaching liquor. Suitable provision may be made for indicating the contents of the vessel, and 60 also for indicating the speed of the vessel.

What I claim is:—

The herein described process of bleaching chemical wood cellulose which consists in placing a concentrated bleaching agent in a 75 rotary vessel, adding water thereto to form a solution, placing within the vessel the cellulose to be bleached in sheet form and dry, and rotating the vessel, the amount of the bleaching solution being so proportioned 80 with respect to the amount of cellulose to be bleached as to render subsequent draining of the bleached cellulose unnecessary.

In witness whereof I have hereunto set my hand in the presence of two witnesses. 85

FREDERICK WILLIAM DOBSON.

Witnesses:

KATHLEEN MARY THOMPSON,  
ERNEST HARKER.